



US008614156B2

(12) **United States Patent**  
**Hess et al.**

(10) **Patent No.:** **US 8,614,156 B2**  
(45) **Date of Patent:** **\*Dec. 24, 2013**

(54) **TEXTILE FABRIC FOR THE OUTER SHELL OF A FIREFIGHTER'S GARMENT**

(75) Inventors: **Diane B. Hess**, Gastonia, NC (US); **Charles A. Thomas**, Pearesburg, VA (US); **Clifton A. Perry**, Charlotte, NC (US); **Richard O. Tucker**, Oakboro, NC (US)

(73) Assignee: **PBI Performance Products, Inc.**, Charlotte, NC (US)

(\*) Notice: Subject to any disclaimer, the term of this patent is extended or adjusted under 35 U.S.C. 154(b) by 0 days.

This patent is subject to a terminal disclaimer.

(21) Appl. No.: **13/275,422**

(22) Filed: **Oct. 18, 2011**

(65) **Prior Publication Data**

US 2012/0034835 A1 Feb. 9, 2012

**Related U.S. Application Data**

(63) Continuation of application No. 10/348,101, filed on Jan. 21, 2003, now Pat. No. 8,071,492, which is a continuation-in-part of application No. 09/933,301, filed on Aug. 20, 2001, now Pat. No. 6,624,096.

(51) **Int. Cl.**

**D03D 15/12** (2006.01)  
**D03D 13/00** (2006.01)  
**D03D 15/00** (2006.01)  
**A62B 17/00** (2006.01)

(52) **U.S. Cl.**

USPC ..... **442/302**; 442/181; 442/203; 442/217;  
428/920; 428/921; 2/458

(58) **Field of Classification Search**  
USPC ..... 442/181-220, 301; 428/920-921  
See application file for complete search history.

(56) **References Cited**

U.S. PATENT DOCUMENTS

|             |         |                  |
|-------------|---------|------------------|
| 2,619,705 A | 12/1952 | Boutwell         |
| 3,347,969 A | 10/1967 | Moelter          |
| 3,511,747 A | 5/1970  | Davies           |
| 3,949,111 A | 4/1976  | Pelletier        |
| 4,048,139 A | 9/1977  | Calundann et al. |

(Continued)

FOREIGN PATENT DOCUMENTS

|    |            |        |
|----|------------|--------|
| CA | 2313995 A1 | 7/2000 |
| CH | 681600 A5  | 4/1993 |

(Continued)

OTHER PUBLICATIONS

Definition of "Polybenzimidazole Fiber (PBI)," Dictionary of Fiber & Textile Technology, Published by Hoechst Celanese, 1990, pp. 115-116.

(Continued)

*Primary Examiner* — Jennifer A Steele

(74) *Attorney, Agent, or Firm* — Hammer & Associates, P.C.

(57) **ABSTRACT**

The present invention is directed to a textile fabric. This fabric is particularly well suited for use as the outer shell fabric of a firefighter's garment. The fabric is a woven or knitted fabric of spun yarns and multi-filament yarns. The spun yarn includes a first staple being a polymer selected from the group consisting of aramid, PBI or PBO or melamine formaldehyde, and a second staple being an aramid polymer. The multi-filament yarn includes an aramid filament.

**19 Claims, 1 Drawing Sheet**



|                          |                              |                                                                                                                                                                        |         |
|--------------------------|------------------------------|------------------------------------------------------------------------------------------------------------------------------------------------------------------------|---------|
| (56)                     | <b>References Cited</b>      | 7,119,036 B2 * 10/2006 Maini .....                                                                                                                                     | 442/197 |
| U.S. PATENT DOCUMENTS    |                              |                                                                                                                                                                        |         |
| FOREIGN PATENT DOCUMENTS |                              |                                                                                                                                                                        |         |
| 4,198,494 A              | 4/1980 Burckel               | DE 4229546 A1 3/1994                                                                                                                                                   |         |
| 4,219,996 A              | 9/1980 Edgawa et al.         | EP 0599587 A1 6/1994                                                                                                                                                   |         |
| 4,469,744 A              | 9/1984 Grot et al.           | FR 2649128 1/1991                                                                                                                                                      |         |
| 4,470,251 A              | 9/1984 Bettcher              | GB 2070077 A 9/1981                                                                                                                                                    |         |
| 4,500,593 A              | 2/1985 Weber                 | JP 1272836 10/1989                                                                                                                                                     |         |
| 4,602,385 A              | 7/1986 Warren                | JP 2191760 7/1990                                                                                                                                                      |         |
| 4,748,065 A              | 5/1988 Tanikella             | JP 2264030 10/1990                                                                                                                                                     |         |
| 4,750,443 A              | 6/1988 Blaustein et al.      | JP 4024240 1/1992                                                                                                                                                      |         |
| 4,865,906 A              | 9/1989 Smith, Jr.            | JP 5125637 5/1993                                                                                                                                                      |         |
| 4,900,613 A              | 2/1990 Green                 | JP 6220730 8/1994                                                                                                                                                      |         |
| 4,923,741 A              | 5/1990 Kosmo et al.          | JP 9078379 3/1997                                                                                                                                                      |         |
| 4,931,345 A              | 6/1990 Böttger et al.        | JP 9119038 5/1997                                                                                                                                                      |         |
| 4,941,884 A              | 7/1990 Green                 | JP 10130990 5/1998                                                                                                                                                     |         |
| 4,958,485 A              | 9/1990 Montgomery et al.     | JP 11279894 10/1999                                                                                                                                                    |         |
| 4,967,548 A              | 11/1990 Fangeat et al.       | JP 2000008247 1/2000                                                                                                                                                   |         |
| 4,996,099 A              | 2/1991 Cooke et al.          | JP 2000045147 2/2000                                                                                                                                                   |         |
| 5,095,549 A              | 3/1992 Aldridge              | JP 2000234236 8/2000                                                                                                                                                   |         |
| 5,119,512 A              | 6/1992 Dunbar et al.         | JP 2000256927 9/2000                                                                                                                                                   |         |
| 5,120,599 A              | 6/1992 Lewis                 | JP 2000273742 10/2000                                                                                                                                                  |         |
| 5,136,723 A              | 8/1992 Aldridge et al.       | JP 2000303285 10/2000                                                                                                                                                  |         |
| 5,177,948 A              | 1/1993 Kolmes et al.         | JP 2000303289 10/2000                                                                                                                                                  |         |
| 5,202,086 A              | 4/1993 Baliga et al.         | RU 2127536 C1 3/1999                                                                                                                                                   |         |
| 5,215,795 A              | 6/1993 Matsumoto et al.      | WO WO 00/66823 11/2000                                                                                                                                                 |         |
| 5,233,821 A              | 8/1993 Weber, Jr. et al.     | WO WO 00/75410 A1 12/2000                                                                                                                                              |         |
| 5,299,602 A              | 4/1994 Barbeau et al.        | WO WO 01/57940 8/2001                                                                                                                                                  |         |
| 5,323,815 A              | 6/1994 Barbeau et al.        | OTHER PUBLICATIONS                                                                                                                                                     |         |
| 5,344,698 A              | 9/1994 Rock et al.           | "Abrade; abrasion," The Random House College Dictionary Revised Edition, The Random House, Inc. (New York), (p. 4,5), (1980).                                          |         |
| 5,447,787 A              | 9/1995 Shaffer               | "Abrasion Resistance," Dictionary of Fiber & Textile Technology, KoSa (Charlotte, NC), (p. 1), (1999).                                                                 |         |
| 5,482,763 A              | 1/1996 Shaffer               | "Tear," The Random House College Dictionary Revised Edition, Random House, Inc. (New York), (p. 1348), (1980).                                                         |         |
| 5,499,663 A              | 3/1996 Barbeau et al.        | "Tear Strength," Dictionary of Fiber & Textile Technology, KoSa (Charlotte, NC), (p. 193), (1999).                                                                     |         |
| 5,538,781 A              | 7/1996 Rao et al.            | Ernest R. Kaswell, "Cover, Copyright pages," Wellington Sears Handbook of Industrial Textiles, Wellington Sears Company, Inc. (New York, NY), p. 154-159, (1963).      |         |
| 5,560,990 A              | 10/1996 Ilg et al.           | Dictionary of Fiber & Textile Technology, Kosa, Charlotte, NC (1999) pp. 42, 44, 184.                                                                                  |         |
| 5,624,738 A              | 4/1997 Barbeau et al.        | NFPA 1971 (2007 Edition), NFPA, 1 Battery Park, Quincy, MA, pp. 1971-33 & 1971-56.                                                                                     |         |
| 5,628,065 A              | 5/1997 Austin                | ASTM D1424-96—Standard Test Method for Tearing Strength of Fabrics by Falling Pendulum Type (Elmendorf) Apparatus, ASTM, 100 Barr Harbor Drive, West Conshohocken, PA. |         |
| 5,637,114 A              | 6/1997 Höhnke                | ASTM D5587-05—Standard Test Method for Tearing Strength of Fabrics by Trapezoid Procedure, ASTM, 100 Barr Harbor Drive, West Conshohocken, PA.                         |         |
| 5,654,067 A              | 8/1997 Dinger et al.         | Re-exam U.S. Appl. No. 90/008132, Amendment filed May 9, 2007.                                                                                                         |         |
| 5,688,594 A              | 11/1997 Lichscheidt et al.   | * cited by examiner                                                                                                                                                    |         |
| 5,691,040 A              | 11/1997 Barbeau et al.       |                                                                                                                                                                        |         |
| 5,701,606 A              | 12/1997 Aldridge             |                                                                                                                                                                        |         |
| 5,858,888 A              | 1/1999 Underwood et al.      |                                                                                                                                                                        |         |
| 5,882,791 A              | 3/1999 van der Werff et al.  |                                                                                                                                                                        |         |
| 5,926,842 A              | 7/1999 Price et al.          |                                                                                                                                                                        |         |
| 5,928,971 A              | 7/1999 Ellis et al.          |                                                                                                                                                                        |         |
| 5,962,627 A              | 10/1999 van der Werff et al. |                                                                                                                                                                        |         |
| 5,983,409 A              | 11/1999 Aldridge et al.      |                                                                                                                                                                        |         |
| 5,996,122 A              | 12/1999 Aldridge et al.      |                                                                                                                                                                        |         |
| 6,038,700 A              | 3/2000 Aldridge et al.       |                                                                                                                                                                        |         |
| 6,065,153 A              | 5/2000 Underwood et al.      |                                                                                                                                                                        |         |
| 6,192,520 B1             | 2/2001 Underwood et al.      |                                                                                                                                                                        |         |
| 6,211,099 B1             | 4/2001 Hutto, Jr. et al.     |                                                                                                                                                                        |         |
| 6,247,179 B1             | 6/2001 Underwood et al.      |                                                                                                                                                                        |         |
| 6,559,079 B1             | 5/2003 Bachner, Jr.          |                                                                                                                                                                        |         |
| 6,562,741 B1             | 5/2003 Lilani                |                                                                                                                                                                        |         |
| 6,624,096 B2             | 9/2003 Thomas et al.         |                                                                                                                                                                        |         |
| 6,699,802 B1             | 3/2004 Hainsworth et al.     |                                                                                                                                                                        |         |
| 6,840,288 B2             | 1/2005 Zhu et al.            |                                                                                                                                                                        |         |
| 6,974,785 B1             | 12/2005 Barbeau et al.       |                                                                                                                                                                        |         |

*Fig. 1**Fig. 2*

## TEXTILE FABRIC FOR THE OUTER SHELL OF A FIREFIGHTER'S GARMENT

### RELATED APPLICATIONS

The instant application is a continuation of U.S. patent application Ser. No. 10/348,101 filed Jan. 21, 2003, which issued as U.S. Pat. No. 8,071,492, which is a continuation-in-part of U.S. patent application Ser. No. 09/933,301 filed Aug. 20, 2001, which issued as U.S. Pat. No. 6,624,096.

### FIELD OF THE INVENTION

The present invention is directed to a textile fabric for use as the outer shell fabric of a firefighter's garment.

### BACKGROUND OF THE INVENTION

The outer shell fabric of a firefighter's garment must be flame, heat, abrasion, tear, and moisture resistant, durable, and lightweight. This outer shell fabric provides the first layer of protection for the firefighter.

U.S. Pat. Nos. 5,095,549; 5,136,723; 5,701,606; 5,983, 409; 5,996,122; and 6,038,700 disclose, among other things, firefighter's garments having an outer shell fabric made of PBI/aramid fibers.

U.S. Pat. No. 5,299,602 discloses a woven, outer shell fabric made for firefighter's garments where the warp yarns are multi-filament aramid yarns and the weft yarns are either multi-filament or spun aramid yarns.

U.S. Pat. No. 5,628,065 discloses a firefighter's hood of a knit fabric formed of a blend of PBI and aramid fibers.

U.S. Pat. Nos. 6,065,153 and 6,192,520 disclose a woven outer shell fabric for a firefighter's garments. This fabric has a plain, twill or rip stop weave and the yarns are a mixture of PBI and aramid fibers. The fabric has a weight ranging from 5.5 to 8 OSY, preferably, 7.5 OSY.

One popular outer shell fabric is a woven fabric of spun yarns consisting of PBI and aramid staple. This fabric is known in the market as 'PBI GOLD®'. In the U.S., this fabric generally is made in the following forms: 1) a 7.5 OSY rip stop weave made from a 16/2 c.c. spun yarns consisting of 40% by weight PBI and 60% by weight of a para-aramid; or 2) a nominal 7.0 OSY (actual 7.3 to 7.4 OSY) rip stop weave made from a 21/2 c.c. spun yarns consisting of 40% PBI and 60% of the para-aramid. Internationally, this fabric is in the form of a 6.0 to 6.5 OSY rip stop weave 24-25/2 c.c. spun yarns of 40% PBI and 60% para-aramid, or a twill weave made from 35/2 c.c. spun yarns of 40% PBI and 60% para-aramid.

Another fabric used as an outer shell fabric is marketed under the trade name 'Millenia' from Southern Mills, Inc. of Union City, Ga. The Millenia fabric is made with a spun yarn consisting of 40% PBO and 60% para-aramid staple.

While 'PBI GOLD®' has proven to be an excellent outer shell fabric, there is still a need to improve these fabrics. There is a desire to have lighter weight fabrics that have better tear and abrasion resistance.

### SUMMARY OF THE INVENTION

The present invention is directed to a textile fabric. This fabric is preferably used as the outer shell fabric of a firefighter's garment. The fabric is a woven or knitted fabric of spun yarns and multi-filament yarns. The spun yarn includes a first staple being a polymer selected from the group consisting of aramid or PBI or PBO or melamine formaldehyde, and a

second staple being an aramid polymer. The multi-filament yarn includes an aramid filament.

### DESCRIPTION OF THE DRAWINGS

For the purpose of illustrating the invention, there is shown in the drawings a form of the invention; it being understood, however, that this invention is not limited to the precise arrangements and instrumentalities shown.

10 FIG. 1 is a plan view of the textile fabric made according to the present invention.

FIG. 2 is a magnified plan view of the textile fabric made according to the present invention.

### DESCRIPTION OF THE INVENTION

15 Referring to the drawings wherein like numerals indicate like elements there is shown in FIG. 1 an illustration of the textile fabric 10 made according to the present invention.

20 Preferably, the fabric 10 has a gold color with a 'checkered' pattern created by black multi-filament yarns 14. The fabric 10 may be woven or knitted. The fabric 10 is preferably woven with spun yarns 12 and multi-filament yarns 14. The weaves are selected from the group consisting of plain, twill, rip stop, and oxford. The fabric weight may range from 6 to 8 OSY, preferably, 7 OSY. The weight ratio of spun yarns to multi-filament yarns should range from 85:15 to 92:8, preferably, 90:10. The multi-filament yarn may be inserted among the spun yarns, in both the warp and weft, at an insertion ratio of 1:5 to 1:20, preferably, 1:9. Preferably, the fabric is treated with a water/moisture resistant finish, as is well known.

25 The spun yarns 12 are a blend of a first staple and a second staple. The first staple is fiber made from a polymer selected from the group of aramid, PBI, PBO, melamine formaldehyde, or combinations thereof. The second staple is a fiber made from an aramid or blends of aramids. Exemplary spun yarns include, but are not limited to, blends of aramid staple, PBI and aramid staple, PBO and aramid staple, melamine formaldehyde and aramid staple, and PBI, PBO, melamine formaldehyde and aramid staple. The spun yarns may have any weight ratio of first and second staples. The weight ratio of first and second staple is preferably 20-60% by weight first staple and 40-80% by weight second staple. The spun yarns most preferably comprise 30-45% by weight of the first staple and 55-70% by weight of the aramid staple. The spun yarns may range in size from 32/2 to 16/2 c.c., preferably, 24/2 c.c.

30 PBI staple fibers are commercially available from Celanese Acetate LLC of Charlotte, N.C. PBO staple fibers are commercially available under the trade name of ZYLON® from 50 Toyobo Co., Ltd. of Osaka, Japan. Melamine formaldehyde fibers are commercially available under the trade name of BASOFIL® from BASF Corporation of Mount Olive, N.J.

35 The aramid staple fibers may be either a meta-aramid or a para-aramid. Such aramid fibers are commercially available 55 under the trade name of TWARON®, CONEX®, and TECHNORA® from Teijin Co. of Osaka, Japan; or NOMEX® or KELVAR® from DuPont of Wilmington, Del.; or P84 from Lenzing AG of Lenzing, Austria; or KERMEL® from Rhodia Inc. of Cranbury, N.J. When the aramid staple fiber forms the second staple mentioned above, it may be either meta-aramid or para-aramid. When the aramid staple fiber forms the second staple mentioned above, it is preferably the para-aramid.

40 The multi-filament yarn is made from aramid filament. Aramid may be either meta-aramid or para-aramid, the para-aramid is preferred. Such aramid fibers are commercially available 60 under the trade name of TECHNORA®, TWARON®, and CONEX® from Teijin Co. of Osaka, Japan,

or NOMEX® or KELVAR® from DuPont of Wilmington, Del., or P84 from Lenzing AG of Lenzing, Austria or KERMEL® from Rhodia Inc. of Cranbury, N.J. The multi-filament yarn ranges in size from 200 to 1500 denier, preferably, 400 denier. The multi-filament yarn may be a flat yarn, a twisted yarn, or a stretch broken yarn.

The instant invention has superior tear and abrasion resistance, at a lower weight, over the PBI GOLD® fabric. The results are set forth in Table 1.

Fabric A is 6.0 OSY fabric; spun yarn is 27/2 c.c. with 45 percent weight PBI and 55 percent Technora® staple; multi-filament is a flat yarn inserted every 10<sup>th</sup> yarn in the warp and weft.

Fabric B is 6.9 OSY fabric; spun yarn is 24/2 c.c. with 45 percent weight PBI and 55 percent Twaron® microdenier staple; multi-filament is a twisted yarn inserted every 9<sup>th</sup> yarn in the warp and weft.

TABLE 1

| Performance Characteristic                      | Test Method                                                    | PBI Gold    | Invention A | Invention B |
|-------------------------------------------------|----------------------------------------------------------------|-------------|-------------|-------------|
| Weight (OSY)                                    |                                                                | 7.5         | 6.0         | 6.8-7.0     |
| Trap Tear (lbs.)                                | ASTM D5733 (Trapezoidal Method)                                | 40 x 35     | 75 x 75     | 63 x 63     |
| Tabor abrasion                                  | ASTM D-3884 (500 g wt. With H18 abrasion wheel)                | 225         | 180         | 293         |
| Thermal Protective Performance, TPP (Composite) | NFPA 1971 (2000 Edition Section 6.10)                          | 40          | 40          | 40          |
| Trap Tear after UV                              | AATCC 16 E (Standard Method for Xenon arc exposure at 1.1 rad) |             |             |             |
| 60 hr                                           |                                                                | 28.4 x 18.7 | 44.6 x 38.5 |             |
| 180 hr                                          |                                                                | 17.8 x 12.3 | 25.7 x 18.9 |             |
| 300 hr                                          |                                                                | 15.2 x 10.6 | 21.2 x 16.1 |             |
| Trap Tear after Sunlight                        | ASTM D5733 (Trapezoid Method)                                  |             |             |             |
| 1 week                                          |                                                                | 30.8 x 20.8 | 64.9 x 62.7 |             |
| 2 week                                          |                                                                | 24.3 x 17.0 | 45.5 x 40.1 |             |
| 3 week                                          |                                                                | 20.0 x 14.6 | 39.0 x 34.2 |             |
| 4 week                                          |                                                                | 18.8 x 13.1 | 34.0 x 33.9 |             |
| 5 week                                          |                                                                | 16.6 x 13.5 | 29.7 x 30.1 |             |
| 6 week                                          |                                                                | 14.8 x 10.5 | 26.6 x 23.6 |             |

The present invention made be embodied in other forms without departing from the spirit and the central attributes thereof and, accordingly, reference should be made to the appended claims, rather than to the foregoing specification, as indicated the scope of the invention.

The invention claimed is:

1. A firefighter garment comprising: an outer shell fabric including a woven material of spun yarns including first staple being a polymer selected from the group consisting of PBI, and/or PBO, and a second staple of an aramid polymer, and multi-filament yarns including a para-aramid filament, and a weight ratio of spun yarn to multi-filament yarn ranges from 85:15 to 92:8.

2. The garment of claim 1 wherein the woven fabric weight ranging from 6 to 8 OSY.

3. The garment of claim 1 wherein the woven fabric has a weave selected from the group consisting plain, twill, rip stop, or oxford.

4. The garment of claim 1 wherein the spun yarn ranges from 32/2 to 16/2 c.c.

5. The garment of claim 1 wherein the multi-filament yarn ranges from 200 to 1500 denier.

10 6. A firefighter garment comprising: an outer shell fabric including a woven material of spun yarn, said spun yarn being a blend of staple, a first staple being made of a polymer selected from the group consisting of PBI, PBO, or combinations thereof and a second staple being made of an aramid, and a multi-filament yarn including para-aramid filaments, said multi-filament yarns being inserted into said woven material, in both the warp and the weft, at a multi-filament 15 yarn to spun yarn ratio of 1:5 to 1:20.

7. The garment of claim 6 wherein said spun yarn being a blend of PBI and aramid staple.

20 8. The garment of claim 6 wherein said spun yarn being a blend of PBO and aramid staple.

9. The garment of claim 6 wherein said spun yarn being a blend of PBI, PBO, and aramid staple.

10 10. A firefighter garment comprising: an outer shell fabric including a woven material of spun yarns including first staple being a polymer selected from the group consisting of aramid, PBI, and/or PBO, and a second staple of an aramid polymer; multi-filament yarns including a para-aramid filament; and a weight ratio of spun yarn to multi-filament yarn ranges from 85:15 to 92:8.

30 11. A firefighter garment comprising: an outer shell fabric including a woven material of spun yarn, said spun yarn being a blend of staple, a first staple being made of a polymer selected from the group consisting of aramid, PBI, PBO, or combinations thereof and a second staple being made of an aramid, and a multi-filament yarn including para-aramid filaments, said multi-filament yarns being inserted into said woven material, in both the warp and the weft, at a multi-filament 35 yarn to spun yarn ratio of 1:5 to 1:20.

12. A firefighter garment comprising: an outer shell fabric 40 including a woven material of spun yarn, said spun yarn being a blend of staple, a first staple being made of an aramid polymer selected from the group consisting of meta-aramid, para-aramid, or combinations thereof and a second staple being made of an aramid polymer selected from the group

45 consisting of meta-aramid, para-aramid, or combinations thereof, and a multi-filament yarn including para-aramid filaments, said multi-filament yarns being inserted into said woven material, in both the warp and the weft, at a multi-filament 50 yarn to spun yarn ratio of 1:5 to 1:20, said woven fabric having a greater trap tear when compared to a fabric of equivalent weight without said filament and a greater tabor abrasion when compared to the fabric of equivalent weight without said filament.

13. A firefighter garment comprising: an outer shell fabric 55 including a woven material of spun yarns including first staple being an aramid polymer selected from the group consisting of meta-aramid, para-aramid, and combinations thereof, and a second staple of an aramid polymer; multi-filament yarns including a para-aramid filament; and a weight ratio of spun yarn to multi-filament yarn ranges from 85:15 to 92:8, said woven fabric having a greater trap tear when compared to a fabric of equivalent weight without said filament and a greater tabor abrasion when compared to the fabric of equivalent weight without said filament.

60 14. A textile fabric comprising: a woven fabric of spun yarns and multi-filament yarns, the spun yarns being in the warp and the weft, the multi-filament yarns being in the warp

and the weft, the spun yarn being a blend of staple selected from the group aramid, PBI, PBO, and combinations thereof, the multi-filament yarn being a para-aramid multi-filament yarn, and a weight ratio of spun yarn to multi-filament yarn ranging from 85:15 to 92:8. 5

**15.** The fabric of claim **14** wherein said spun yarn having a cotton count in the range of 32/2 to 16/2.

**16.** The fabric of claim **14** wherein said multi-filament yarns being inserted into said woven material, in both the warp and the weft, at a multi-filament yarn to spun yarn ratio 10 of 1:5 to 1:20.

**17.** A firefighter garment comprising an outer shell fabric according to claim **14**.

**18.** A firefighter garment comprising: an outer shell fabric including a woven material of spun yarns including first 15 staple being a polymer selected from the group consisting of PBI, and/or PBO, and a second staple of an aramid polymer, and multi-filament yarns including a filament having a tenacity of at least 22 grams per denier, and a weight ratio of spun yarn to multi-filament yarn ranges from 85:15 to 92:8. 20

**19.** A textile fabric comprising: a woven fabric of spun yarns and multi-filament yarns, the spun yarns being in the warp and the weft, the multi-filament yarns being in the warp and the weft, the spun yarn being a blend of staple selected from the group aramid, PBI, PBO, and combinations thereof, 25 the multi-filament yarn comprising a filament having a tenacity of at least 22 grams per denier, and a weight ratio of spun yarn to multi-filament yarn ranging from 85:15 to 92:8.

\* \* \* \* \*